

## UNITED STATES PATENT OFFICE

JOHN MURSCH, OF TEANECK, NEW JERSEY, ASSIGNOR TO JOSEPH GATTI, OF NEW YORK, N. Y.

## METHOD OF PRODUCING SHEETED COMPOUNDS

No Drawing.

Application filed April 29, 1931. Serial No. 533,795.

The present invention relates to the production of sheet materials from compounds employing waste fibre such as newsprint, rags or the like, combined with a binding material in the nature of a synthetic resin. 5  
In the broadest aspect of my invention, I propose to initially prepare the waste fibre, as waste newsprint, in a dry form, this initial preparatory step consisting in the reduction of the material to a state of comparatively uniform sub-division, as in a hammer mill. I next propose to thoroughly and effectually impregnate the complete fibrous mass with uncured resin, either by application of the resin in the form of a liquid varnish, or by developing the resin from liquid ingredients within the fibrous mass itself. Having thus secured a complete impregnation of the mass, I may reduce a mass which 10 is either dry or in a plastic condition to a form in which it may flow as a liquid, this reduction being accomplished preferably through the addition of a sufficient amount of water to dilute the mass and separate the fibres. This loosening of the fibres after the 15 addition of water may be accomplished by a relatively gentle agitation or mixing to separate the fibres without destroying or breaking up the fibres themselves, or removing more than a minimum amount of impregnating material therefrom. With the mass reduced to a condition in which it can flow as a liquid, I am enabled to deliver the liquid or semi-liquid material on to a screen such as employed in the production of paper, spreading the liquid in a film of uniform thickness thereover. With the screen so coated with a uniform depth of material, the production of a vacuum in a manner which will be obvious 20 to those skilled in the art, withdraws surplus liquid, as water, and converts the mass into a coherent sheet, which may thereafter be treated either for the production of molded products, or in sheet form as board. In 25 either case the uncured sheet is subjected to curing temperatures which convert the resins into an insoluble product having the waste fibre as an essential ingredient. By suitably altering the proportions of fibre to resin and 30 controlling the degree of sub-division of the

dry fibre, the resulting product may be varied within desired limits, the type and character of the finish depending in part, at least, upon the proportions employed.

According to one method of practicing the invention which has resulted in suitable products, I first reduce the waste paper or the like, which may be in the form of newsprint or book-paper, into a finely ground condition through the employment of a hammer mill. This hammer mill is a familiar article of commerce, and comprises rotating hammers which are capable of beating out and grinding the loose dry mass of paper into finely divided form. Having thus prepared the fibre for impregnation with the resin material, I prefer to develop the resin directly in the fibre itself, and to this end I thoroughly mix at room temperatures the following proportions of material:

|                           |    |
|---------------------------|----|
| 2 pounds of paper         | 70 |
| 7 pounds of formaldehyde  |    |
| 7 pounds of cresylic acid |    |
| 2 pounds of caustic soda  |    |
| 8 pounds of water         | 75 |

The acid and caustic soda are caused to thoroughly penetrate the fibre and thereafter the water is added. The operation is preferably carried out in a steam-heated kettle at five 80 to ten pounds steam pressure, the resin developing directly within the fibre.

When the reaction has been completed, it will be found that the resulting mixture is somewhat plastic, and that the individual 85 fibres are thoroughly and effectually impregnated with the uncured resin. To this material may be added a sufficient amount of water to make the resulting material flowable, and permit its being delivered or flowed on 90 to a vacuum screen in the form of a sheet.

As an alternative method of producing the impregnated fibre, I may mix the dry, finely divided waste paper or the like with a liquid resin varnish. In this case the dry waste and 95 resin varnish are thoroughly mixed to secure as nearly a uniform impregnation of the dry ingredients as possible. Having thus impregnated the material, it is dried below curing temperatures, if desired, and to this ma- 100

terial may be added a sufficient amount of water to dilute and cause it to flow, this reduction to a flowable condition being preferably accomplished through agitation. Although this method of producing a wet, flowable mass may conceivably be employed, nevertheless it is not as effective as the method previously described, which results in the development of the resin directly within the fibre itself. This is due to the fact that impregnation of the fibre is more complete and uniform in the first method, and in the second place less of the resinous material is removed from the fibre with the added water with the first method than with the second.

With either method of production, the wet, mobile, flowable mass is delivered to a screen and a vacuum drawn therethrough for removing the surplus water and other liquids, and converting the mass into a reasonably dry, coherent sheet. This sheet may be cut into proper form and the cut portions inserted in a mold and subjected to curing temperatures and pressures, whereby molded articles are produced, or it may be cured directly in sheet form, the finish in either case depending to some extent upon the proportions of synthetic resin to the proportions of fibre which are employed. By reducing the impregnated fibre to a liquid or semi-liquid condition and converting it into a coherent sheet from this form, it is found that the resulting product when cured is much improved as compared with the product produced directly from the impregnated fibre in a dry, loose condition, this fibre being placed directly into a mold and then subjected to curing temperatures and pressures.

As an alternative to the formation of the coherent sheet on the vacuum screen, the liquid mass can be drawn off on the felt vacuum rolls of paper machines of the wet type. Regardless of whether the sheets are prepared on a vacuum screen or felt, the drying is subsequently completed in an oven or with steam-heated racks. The heat employed in the subsequent drying operation is merely sufficient to dry off moisture without promoting any curing of the resin. This semi-cured sheet, as it may be termed, merely requires curing temperatures combined with whatever pressure may be desired to provide a finished product with a hard, smooth surface.

What is claimed is:

1. The method of producing sheeted compounds which consists in reducing dry waste fibre to a finely divided condition, thoroughly impregnating the divided fibre with an uncured resin, reducing the impregnated fibrous mass to a flowable condition, forming a uniform film of the flowable mass, and drying into a coherent sheet.

2. The method of producing sheeted compounds which consists in reducing dry waste fibre to a finely divided condition, thorough-

ly impregnating the divided fibre with an uncured resin, reducing the impregnated fibrous mass to a flowable condition, forming a uniform film of the flowable mass, drying into a coherent sheet, and finally subjecting the sheet or a part thereof to temperatures sufficiently elevated to cure the resin.

3. The method of producing sheeted compounds which consists in reducing dry waste fibre to a finely divided condition, thoroughly impregnating the divided fibre with an uncured resin, reducing the impregnated fibrous mass to a flowable condition, delivering the liquid mass on to a screen, and drying the mass into a coherent sheet through vacuum.

4. The method of producing sheeted compounds which consists in reducing dry waste fibre to a finely divided condition, developing a synthetic resin directly within the mass of fibre to produce a somewhat plastic mass, reducing the mass through the addition of water and mixing to a flowable condition, forming a film while in this condition, and drying the film to produce a coherent sheet of fibre impregnated with uncured resin.

5. The method of producing sheeted compounds which consists in reducing dry waste fibre to a finely divided condition, developing a synthetic resin directly within the mass of fibre to produce a somewhat plastic mass, reducing the mass through the addition of water and mixing to a flowable condition, forming a film while in this condition, drying the film to produce a coherent sheet of fibre impregnated with uncured resin, and curing the sheeted material at a temperature sufficiently high to convert the resin into an insoluble material.

In testimony whereof I have signed my name to this specification.

JOHN MURSCH.

105

110

115

120

125

130